

1

3,393,041

**MULTILAYER SILVER HALIDE ELEMENTS CONTAINING THIAZOLE COLOR COUPLERS FOR YELLOW**

Marcel Hendrik Verbrugghe, Wilrijk-Antwerp, and Arthur Henri De Cat and Raymond Albert Roosen, Mortsel-Antwerp, Belgium, assignors to Gevaert Photo-Produc-  
tuen N.V., Mortsel, Belgium, a company of Belgium  
No Drawing. Filed July 8, 1964, Ser. No. 381,260  
Claims priority, application Belgium, July 9, 1963,  
Patent 634,670

7 Claims. (Cl. 96—74)

**ABSTRACT OF THE DISCLOSURE**

Improved color couplers for use primarily in photographic multilayer color materials are described. The color couplers are 2-(aryloyacetamido)-thiazoles having at least one sulphonic acid group on the aryl moiety. The color couplers when employed in photographic materials exhibit an unusually high degree of stability to the action of light, heat and humidity.

This invention is concerned with the production of photographic color images, with the color couplers for yellow utilised therein and with photographic materials comprising such color couplers.

With respect to the production of a photographic color image in a light-sensitive silver halide emulsion layer it is known that the exposed silver halide is developed to a silver image with the aid of an aromatic primary amino compound in the presence of a color coupler by which at the areas corresponding with the silver image a dye is formed by reaction with the oxidised developing substance.

In subtractive color photography use is made currently of a light-sensitive photographic color material comprising a silver halide emulsion layer sensitised to red light, a silver halide emulsion layer sensitised to green light and a silver halide emulsion layer sensitised to blue light, in which emulsion layers are formed a cyan, a magenta, and a yellow dye image by using appropriate color couplers during the color development.

It is known that color couplers must satisfy various requirements according to the method by which the color material is manufactured and the purpose for which it is used.

For manufacturing an appropriate photographic multilayer color material containing color couplers for each color separation image in the differently optically sensitised silver halide emulsion layers, the color couplers ought to be present in the hydrophilic silver halide emulsion layers in non-migratory form. This object can be accomplished e.g. by the use of a sufficiently water-soluble color coupler comprising an organic radical sufficiently large to prevent the color coupler from diffusing in the hydrophilic silver halide emulsion layer, or by the utilisation of a lipophilic color coupler, which in dissolved state in a high-boiling organic solvent is dispersed in the silver halide emulsion layer.

2

In the production of color images, more particularly of positive color images e.g. on a paper support, it is important to dispose of color couplers, which on color development form dyes that are quite resistant to the action of light, humidity, and heat.

5 A new class of color couplers for yellow of the keto-methylene type, more particularly 2-(aryloyacetamido)-thiazole derivatives has been found now. These color couplers display a high activity during color development and form yellow dyes possessing a favorable resistance to humidity and heat.

These 2-(aryloyacetamido)-thiazole derivatives are characterised by the presence of at least one group solubilising in water, more particularly a sulphonic acid group in the aryl part of the molecule. The sulphonic acid group(s) can be implanted directly in the aromatic nucleus of the aryl group or can be present in an aromatic nucleus, which is linked to the aromatic nucleus of the aryl group by means of a bivalent radical.

15 Suitable color couplers for yellow according to the present invention are color couplers in which at least one sulphonic acid group is implanted directly in the aromatic nucleus of the aryl group, and which comply with the following general formula:

25



30 wherein:

R<sub>1</sub> represents a sulphonic acid group or its salt form,  
R<sub>2</sub> represents hydrogen, halogen, alkoxy, a sulphonic acid group or its salt form, or a group rendering fast to diffusion such as a n-hexadecyloxy group,

35 R<sub>3</sub> represents hydrogen, alkyl, substituted alkyl, aryl, substituted aryl, preferably a group rendering fast to diffusion such as i.e. the group —X—R, in which X represents a chemical bond, oxygen or sulphur and R an acyclic aliphatic hydrocarbon rest with 5 to 20 carbon atoms,

40 R<sub>4</sub> represents hydrogen, alkyl, substituted alkyl, aryl, a substituted aryl radical with substituents such as alkoxy, halogen, alkylsulphonyl, a group rendering fast to diffusion such as a n-hexadecyloxy group, a n-hexadecylmercapto group or a pentadecyl group, and

45 R<sub>3</sub> and R<sub>4</sub> together may represent the atoms necessary for completing an aromatic ring system, which is either or not further substituted.

50 Suitable color couplers for yellow according to the present invention are color couplers, in which at least one sulphonic acid group in the aryl part of the molecule is implanted in an aromatic nucleus linked to the aromatic nucleus of the aryl group by means of a bivalent radical, and which comply with the following general Formula II

55



wherein:

R<sub>2</sub>, R<sub>3</sub> and R<sub>4</sub> have the same significance as given in Formula I,

R'<sub>1</sub> represents an either or not further substituted sulphonated aromatic radical such as e.g. a sulphonated phenyl group, and

Y represents a bivalent radical such as a —CONH— group, a —SO<sub>2</sub>NH— group, or a —NHCONH— group.

The preparation of the color couplers according to the general Formula I is illustrated by the following reaction scheme:



thiazole hydrobromide is formed. The base is set free therefrom by treatment with concentrated ammonium hydroxide. A white crystalline product is obtained after separating the precipitate, rinsing with water and recrystallising from ethanol. Melting point: 109° C.

#### 2-AMINO-4-METHYL-5-TETRADECYLTHIAZOLE

To an amount of methyl pentadecyl ketone dissolved in carbon tetrachloride is added dropwise an equivalent amount of bromine at 15-20° C. while stirring. The bromine immediately reacts and a vigorous development of hydrobromic acid takes place. The mixture is stirred for 30 min. yet the solvent is then distilled off in vacuo. The residue is dissolved in ethanol and an equivalent amount of thiourea is added. Subsequently the reaction mixture is heated for 30 min. at reflux temperature and then neutralised with ammonium hydroxide. The mixture is then poured out into ice water. The resulting precipitate is dried and recrystallised from n-hexane. A white finely crystalline product is obtained. Melting point: 57° C.

#### 2-AMINO-4-PHENYL-5-TETRADECYLTHIAZOLE

To an amount of palmitoylbenzene (F. Krafft, Ber. 19 (1886) 2983) dissolved in carbon tetrachloride is added dropwise an equivalent amount of bromine whilst stirring. The brown color of bromine immediately disappears and a vigorous development of hydrobromic acid takes place. The mixture is stirred for another 30 min. and subsequently the solvent is distilled off in vacuo. The residue is recrystallised from ethanol. White crystal leaflets of  $\alpha$ -bromopalmitoylbenzene are obtained. Melting point: 47-48° C.

To an amount of this compound dissolved in ethanol is added an equivalent amount of thiourea and the resulting reaction mixture is heated at boiling temperature for 1 h. After neutralisation of the reaction mixture with ammonium hydroxide and pouring out in water, the resulting precipitate is rinsed with water and dried. After recrystallisation from n-hexane the 2-amino-4-phenyl-5-tetradecylthiazole is obtained in the form of a white crystalline product. Melting point: 68° C.

#### 2-AMINO-4-(4'-METHOXYPHENYL)-5-TETRADECYLTHIAZOLE

This compound is synthesised in a similar way as described in the foregoing preparation starting, however, with 4-palmitoyl anisol.

4-palmitoyl anisol is prepared by Friedel-Crafts acylation with palmitoyl chloride as described in F. Krafft, Ber. 19 (1886) 2983. After recrystallisation from ethanol a white crystalline product is obtained. Melting point: 70° C.

4-( $\alpha$ -bromopalmitoyl)-anisol is obtained in the form of white crystalline leaflets after recrystallisation from ethanol. Melting point: 79-80° C.

2 - amino - 4 - (4' - methoxyphenyl) - 5 - tetradecylthiazole is obtained as a white crystalline product after recrystallisation from n-hexane. Melting point: 79° C.

#### 2-AMINO-4-( $\alpha$ -CARBETHOXYHEPTADECYL)-THIAZOLE

First the  $\alpha$ -n-hexadecyl acetylacetate ethyl ester is prepared analogously to the methyl ester (J. Gunther Ber. 71 B (1938) 2634) starting with acetylacetate ethyl ester, n-hexadecyl bromide and sodium ethylate in ethanol. A colourless viscous oil is obtained. Boiling point: 174-175° C. (0.5 mm. Hg).

To a solution of this  $\alpha$ -n-hexadecyl acetylacetate ethyl ester in carbon tetrachloride is added dropwise an equivalent amount of bromide. This solution is kept at

room temperature for 24 h. By caralysis of the formed hydrobromic acid the initially  $\alpha$ -bromo-substituted  $\alpha$ -n-hexadecyl acetylacetate ethyl ester is converted into the  $\gamma$ -bromo derivative. The solvent is then distilled off in vacuo and the residue is dissolved in ethanol. Subsequently an equivalent amount of thiourea is added and the reaction mixture is heated at boiling temperature for 15 min. The base is set free from the resulting amino-thiazole hydrobromide by treatment with ammonium hydroxide. After pouring out in water, the resulting precipitate is dried and recrystallised from n-hexane. The 2-amino-4-( $\alpha$ -carbethoxyheptadecyl)-thiazole is obtained in the form of white fine crystal needles. Melting point: 90° C.

#### 2-AMINO-5-n-HEXADECYL MERCAPTOOTHIAZOLE

To a solution of 2-amino-5-bromothiazole hydrobromide (J. P. English, J. Am. Chem. Soc. 68 (1946) 456) in a mixture of ethanol and water (10:1) is dropwise added an equivalent amount of n-hexadecylmercaptane and a double amount of potassium hydroxide dissolved in ethanol. The reaction mixture is heated to boiling temperature and stirred at this temperature for 4 h. The formed potassium bromide is filtered off. When cooling a precipitate is formed in the filtrate. This precipitate is first recrystallised from dichloroethane and secondly from methanol. A yellowish crystalline product is obtained. Melting point: 98° C.

#### 2-aminothiazole

2-amino-4-phenylthiazole (Dodson, King J.A.C.S. 67, 2242 (1945)).

#### 2-aminobenzothiazole

(b) Preparation of 2-benzoylacetamido)-thiazole derivatives.—Reaction step (a)

#### GENERAL PROCESS

0.1 mole of amino derivative, 0.1 mole of  $\beta$ -ketoester derivative and 0.2 g. of anhydrous sodium acetate are added to 100 ml. of anhydrous xylene. The reaction mixture is refluxed and a mixture of xylene and the formed ethanol is distilled off slowly till the temperature reaches 138° C., which lasts approximately one hour.

Subsequently the remaining xylene is distilled off in vacuo. To the residue 200 ml. of hexane are added and the resulting precipitate is filtered off and recrystallised from a suited solvent.

The results of condensations of 2-aminothiazole derivatives with fluorosulphonyl-substituted  $\beta$ -ketoester derivatives are listed in Table 1 (col. 3 and 4).

(c) Alkaline hydrolysis to sulphonic acid derivatives of the fluorosulphonyl-substituted benzoylacetanilides.—Reaction step (b)

#### GENERAL PROCESS

0.1 mole of sulphonylfluoride derivative is heated to boiling temperature with 400 ml. of acetone. Whilst stirring 60 ml. of 5 N sodium hydroxide are added slowly, thus causing an exothermic reaction. The reaction mixture is heated at boiling temperature for 30 min. whilst stirring. Subsequently the mixture is acidified with acetic acid and next cooled to room temperature. The resulting precipitate is washed with water and recrystallised from a suited solvent.

The results of these alkaline hydrolyses are listed in Table 1 (col. 5 and 6). Col. 6 refers to the number of the structural formula of the prepared color coupler for yellow, whereas col. 7 indicates the absorption maximum of the azomethine dye obtained when developing with N-diethyl-p-phenylene diamine.

TABLE 1

| Utilised amino derivative |                             | Utilised $\beta$ -ketoester derivative | Fluorosulphonyl substituted 2-(benzoyl acetamide)-thiazole | Sulphonic acid derivative (sodium salt) |                          |                               |                                                    |
|---------------------------|-----------------------------|----------------------------------------|------------------------------------------------------------|-----------------------------------------|--------------------------|-------------------------------|----------------------------------------------------|
|                           |                             |                                        | Recrys-talisation medium                                   | Melt-ing point, °C.                     | Recrys-talisation medium | Number of struc-tural formula | Absorp-tion max-imum of the azo-methine dye, $\mu$ |
| $R_3=H$                   | $R_4=$                      | $FO_3S$                                | Acetone..... 102-104                                       | Ethylene-glycol mono-ether.             | 1                        | 465                           |                                                    |
| $R_3=-C_{14}H_{29}$       | $R_4=-CH_3$                 | $FO_3S$                                | Benzene/ hexane. 104                                       | Ethanol/ water.                         | 2                        | 457                           |                                                    |
| $R_2=-C_{14}H_{29}$       | $R_4=$                      | $FO_3S$                                | Aceto-nitrile. 70                                          | do.....                                 | 3                        | 465                           |                                                    |
| $R_3=-C_{14}H_{29}$       | $R_4=$                      | $FO_3S$                                | Methanol.... 70                                            | do.....                                 | 4                        | 465                           |                                                    |
| $R_3=H$                   | $R_4=-CH(COOH)C_{16}H_{33}$ | $FO_3S$                                | Hexane..... 79                                             | do.....                                 | 5                        | 460                           |                                                    |
| $R_3=-SC_{16}H_{33}$      | $R_4=H$                     | $FO_2S$                                | Dichloro-ethane. 150                                       | do.....                                 | 6                        | 465                           |                                                    |
| $R_3=-C_{14}H_{29}$       | $R_4=$                      | $FO_2S$                                | Benzene.... 102-303                                        | Methanol....                            | 7                        | 450                           |                                                    |
| $R_3=H$                   | $R_4=H$                     | $FO_2S$                                | Dioxan..... 183                                            | Isopropanol/ water.                     | 8                        | 455                           |                                                    |
| $R_3=H$                   | $R_4=$                      | $FO_2S$                                | .....do..... 152                                           | Dioxan/ ethanol.                        | 9                        | ±465                          |                                                    |
| $R_3=H$                   |                             | $FO_2S$                                | .....do..... 150                                           | Ethanol/ water.                         | 10                       | 465                           |                                                    |
| $R_3$<br>$R_4$<br>        |                             |                                        |                                                            |                                         |                          |                               |                                                    |

Specific examples of color couplers for yellow according to the present invention in which a sulphonic acid group in the aroyl part of the molecule is linked to an

aromatic nucleus which is linked by a bivalent radical to the aromatic nucleus of the aroyl group, comply with the following structural formulae:



The following reaction scheme illustrates the synthesis of these compounds:

is carried out in dioxan at 80° C. under a hydrogen pressure of 42 kg. per sq. cm. When the calculated amount

(a')



(I')

(b')



(II')

(c')



(III')

(d')



wherein:

Z represents a —COCl group or a —NCO group, and W stands for a —CO— group or a —NHCO— group.

50

(A) Utilized starting products

(a) 2-[α-3'-aminobenzoyl]acetyl]-amino-4-(p-n-hexadecyloxyphenyl)-thiazole

55



The synthesis of 2-[α-(3'-nitrobenzoyl)-acetyl]amino-4-(p-n-hexadecyloxyphenyl)-thiazole (reaction step (a')) is similar to that of the analogous condensation products described in the copending patent application for "Color Couplers for Color Photography." A yellow crystalline product is obtained by condensation of 41.6 g. of 2-amino-4-(p-n-hexadecyloxyphenyl)-thiazole with 23.7 g. of 3-nitrobenzoyl acetic acid ethyl ester and by recrystallisation from dioxan. Melting point: 135° C.

65

The resulting nitro derivative is then converted into the amine by hydrogenation in the presence of Raney nickel as a catalyst (reaction step (b')). The reduction

of hydrogen is consumed, the catalyst is filtered off. On cooling a precipitate is formed in the filtrate. This precipitate is collected and washed with dichlorethane. The 2-α-(3'-aminobenzoyl)-acetylamino-4-(p-n-hexadecyloxyphenyl)-thiazole is obtained in the form of a white to brownish crystalline product. Melting point: 157-158° C.

(b) 3-fluorosulphonyl benzoyl chloride is prepared as described in the above-mentioned Belgian patent specification.

(c) 3-fluorosulphonyl phenyl isocyanate is prepared as described in the above-mentioned Belgian patent specification.

(B) Reaction of 2-α-(3'-aminobenzoyl)-acetylamino-4-(p-n-hexadecyloxyphenyl)-thiazole with fluorosulphonyl compounds.—Reaction step (c')

(a) With 3-fluorosulphonyl benzoyl chloride.—The synthesis is similar to that stated in the above-mentioned patent specification. When starting with 11.54 g. of the thiazole derivative mentioned under B and an equivalent amount of 3-fluorosulphonyl benzoyl chloride a yellowish finely grained product is obtained finally after recrystallisation from a mixture of ethanol and methanol. Melting point: 166° C.

(b) With 3-fluorosulphonyl phenyl isocyanate.—The synthesis is similar to that stated in the above-mentioned patent specification. When starting with 11.54 g. of thia-

75

zole derivative and an equivalent amount of 3-fluorosulphonyl phenyl isocyanate a yellowish crystalline product is obtained after recrystallisation from acetonitrile. Melting point: 180° C.

(C) Alkaline hydrolysis to sulphonic acid derivatives.—  
Reaction step (d')—

The alkaline hydrolysis of the sulphonyl fluoride derivatives prepared according to reaction step (c') is carried out as stated under 2(c). The results of specific alkaline hydrolysis are listed in Table 2.

a blue-sensitive silver halide emulsion layer with a color coupler for yellow. The support of this multilayer material may consist of paper, glass, cellulose nitrate, a cellulose ester such as cellulose triacetate, polyester, polystyrene or another synthetic or natural resin.

5 A yellow filter layer generally comprising colloidal silver dispersed in gelatin, is provided usually between the silver halide emulsion layer containing a color coupler for yellow and the green-sensitised silver halide emulsion layer.

10 As sulphonyl fluoride derivatives the color couplers for

TABLE 2

| Sulphonyl fluoride derivative |                                                                                                                                  | Sulphonic acid derivative (SO <sub>3</sub> Na) |                                                       |
|-------------------------------|----------------------------------------------------------------------------------------------------------------------------------|------------------------------------------------|-------------------------------------------------------|
|                               |                                                                                                                                  | Recrystallisation medium                       | Number of the structural formula of the color coupler |
| FSO <sub>2</sub>              | XNH—C <sub>6</sub> H <sub>4</sub> —COCH <sub>2</sub> CONH—S—N=C—C <sub>6</sub> H <sub>4</sub> —O—C <sub>16</sub> H <sub>33</sub> | Ethylene glycol mono-methyl ether/water.       | 11                                                    |
| —NHCO—                        | do                                                                                                                               | do                                             | 12                                                    |

The color couplers need not necessarily be separated in the form of sulphonic acid derivatives before their addition to the silver halide emulsion. The sulphonic acid derivatives formed "in situ" from the sulphonyl fluoride derivatives by dissolving the latter derivatives in alkali may be added as such to the emulsion. Preferably 1 mole of sulphonyl fluoride derivative is dissolved therefor in an aqueous solution of 3 mole of sodium hydroxide and after adjustment of the pH value in accordance with the pH of the emulsion applied the resulting clear solution is added in the form of a 5 to 10% aqueous solution to the silver halide emulsion.

During the preparation of the light-sensitive color material the non-migratory color couplers for yellow according to the above-mentioned general formulae are mixed homogeneously in dissolved state with the light-sensitive silver halide emulsion preferably immediately before the coating of the emulsion. This may as well be added to the composition of a water-permeable non-light-sensitive layer, which is in direct contact with the light-sensitive silver halide emulsion layer or they may be incorporated into a non-light-sensitive layer which is separated from the light-sensitive layer by a water-permeable non-light-sensitive layer. The silver halide emulsion contains the usual colloids such as gelatin, poly (vinyl alcohol), collodion or other suitable natural or synthetic colloids. The photographic emulsion may further contain usual ingredients such as hardeners, chemical sensitising agents, optical sensitising agents, plasticisers, development accelerators, stabilising agents and wetting agents.

The color couplers for yellow described in the present invention are added usually to a blue-sensitive silver halide emulsion. According to a common procedure in the art this silver halide emulsion is coated as the last color coupler-containing layer of a photographic multilayer color material. Such photographic multilayer color material usually consists in the given sequence of a support, a red-sensitised silver halide emulsion layer with a color coupler for cyan, a green-sensitised silver halide emulsion layer with a color coupler for magenta and

yellow according to the present invention may be applied in so-called "droplet emulsions" (cf. U.S. patent specification 2,304,940).

For the production of photographic color images according to the present invention an exposed silver halide emulsion layer is developed with an aromatic primary amino developing substance in the presence of a color coupler for yellow according to the present invention.

40 All color developing agents capable of forming azomethine dyes can be utilised as developers. Aromatic primary amino compounds such as p-phenylene diamine and derivatives such as N-diethyl-p-phenylene diamine, N,N - diethyl-N'-sulphomethyl-p-phenylene diamine and N,N-diethyl-N'-carboxymethyl-p-phenylene diamine are commonly used.

45 On color development with aromatic primary amines such as N-diethyl-p-phenylene diamine the color couplers for yellow according to the present invention form yellow dyes having an absorption spectrum which makes these color couplers apt to be used i.a. in positive material (absorption maximum from 450 to 465 m $\mu$ ).

50 These color couplers manifest a high activity during the development, i.e. they furnish color images having high color density.

55 The dyes formed on color development show good resistance to heat and humidity. This is illustrated by comparative tests, the description and results of which will be given hereinafter.

60 The resistance to humidity and heat of the dyes is determined from the decrease in density of a developed wedge print after having stored said wedge print for a certain time (e.g. 5 days) at a specific temperature (e.g. 35° C.) and a relative humidity (e.g. 87%) while being protected from light.

65 The following table clearly illustrates the resistance to humidity and heat of dyes formed on color development by reaction of the resulting oxidation product of N-diethyl-p-phenylene diamine with color couplers according to the present invention and of a color coupler described in the British patent specification 873,125.

| Formula of the color coupler | Maximum density at the beginning of the test | Maximum density after 5 days at 35° C. and a relative humidity of 87% | The percentage decrease of maximum density after 5 days at 35° C. and at a relative humidity of 87% |
|------------------------------|----------------------------------------------|-----------------------------------------------------------------------|-----------------------------------------------------------------------------------------------------|
|                              | 1.2                                          | 1.2                                                                   | 0                                                                                                   |
|                              | 1.2                                          | 1.2                                                                   | 0                                                                                                   |
|                              | 1.2                                          | 0.9                                                                   | 25                                                                                                  |

(Color coupler for yellow according to the British Patent Specification 783,887)

The higher activity during color development of color couplers according to the present invention is proved by a comparative test in which a similar amount of color coupler for yellow is added to two identical silver halide emulsions, i.e. a color coupler A according to the present invention and a color coupler B containing no thiazole group, more particularly a color coupler for yellow stated in the British patent specification 783,887.

These silver halide emulsions are coated, exposed and developed in identical conditions. The relative maximum density of the developed emulsion strips comprising the color coupler A and B respectively listed in the following table.

30 35 40 45

iod layer adjacent to said light-sensitive silver halide emulsion layer a color coupler for yellow which is a 2-(aryloxyacetamido)-thiazole, wherein at least one sulfonic acid group is present in the aryl part of the molecule.

3. Photographic multilayer color material comprising three silver halide emulsion layers which have different optical sensitivities, and containing in non-migratory form in a member selected from the blue-sensitive silver halide emulsion layer and a non-light-sensitive water-permeable colloid layer adjacent thereto a color coupler for yellow which is a 2-(aryloxyacetamido)-thiazole wherein at least one sulfonic acid group is present in the aryl part of the molecule.

| Color coupler | Maximum density |
|---------------|-----------------|
| A....         | 200             |
| B....         | 165             |

As to the structure of the color couplers according to the present invention, it should be noticed yet that when using the expression "sulphonic acid group" or "sulphonic acid substituent" the acid form as well as the salt form of this group or substituent are meant and that whenever the color couplers are used in the salt form they preferably contain an alkali metal cation, an ammonium group or an amine salt group as a cation.

60 65 70 75

We claim:

1. Photographic material comprising a silver halide emulsion layer and a color coupler for yellow which is a 2-(aryloxyacetamido)-thiazole wherein at least one sulfonic acid group is present in the aryl part of the molecule.

2. Photographic multilayer color material containing in non-migratory form in a member selected from the group consisting of a light-sensitive silver halide emulsion layer and a non-light-sensitive water-permeable col-

4. Photographic multi-layer color material containing in non-migratory form in a member selected from the group consisting of a light-sensitive silver halide emulsion layer and a non-light-sensitive water-permeable colloid layer adjacent to said light-sensitive silver halide emulsion layer a color coupler for yellow having the general formula:



wherein

$\text{R}_1$  represents a member selected from the group consisting of a sulfonic acid group and a salt form thereof;  
 $\text{R}_2$  represents a member selected from the group consisting of a hydrogen atom, a halogen atom, a methoxy

group, a sulfonic acid group, a sulfonic acid salt group, and a group rendering fast to diffusion,  
 R<sub>3</sub> represents a member selected from the group consisting of a hydrogen atom, an alkyl group, an aryl group, and a group rendering fast to diffusion,  
 R<sub>4</sub> represents a member selected from the group consisting of a hydrogen atom, an alkyl group, an aryl group, and a group rendering fast to diffusion,  
 further R<sub>3</sub> and R<sub>4</sub> together may also represent the atoms necessary for completing an aromatic ring system.

5. Photographic multi-layer color material containing in non-migratory form in a member selected from the group consisting of a light-sensitive silver halide emulsion layer and a non-light-sensitive water-permeable colloid layer adjacent to said light-sensitive silver halide emulsion layer a color coupler for yellow having the general formula:



wherein

R<sub>2</sub> represents a member selected from the group consisting of a hydrogen atom, a halogen atom, a methoxy group, a sulfonic acid group, a sulfonic acid salt group, and a group rendering fast to diffusion,  
 R<sub>3</sub> represents a member selected from the group consisting of a hydrogen atom, an alkyl group, an aryl group, and a group rendering fast to diffusion,  
 R<sub>4</sub> represents a member selected from the group consisting of a hydrogen atom, an alkyl group, an aryl group, and a group rendering fast to diffusion,  
 Y represents a bivalent radical, and  
 R' represents a sulphonated aromatic radical.

6. Photographic multi-layer color material comprising three silver halide emulsion layers which have different optical sensitivities, and containing in non-migratory form in a member selected from the blue-sensitive silver halide emulsion layer and a non-light-sensitive water-permeable colloid layer adjacent thereto a color coupler for yellow having the general formula:



wherein

R<sub>1</sub> represents a member selected from the group consisting of a sulfonic acid group and a salt form thereof,  
 R<sub>2</sub> represents a member selected from the group consisting of a hydrogen atom, a halogen atom, a methoxy

group, a sulfonic acid group, a sulfonic acid salt group, and a group rendering fast to diffusion,  
 R<sub>3</sub> represents a member selected from the group consisting of a hydrogen atom, an alkyl group, an aryl group, and a group rendering fast to diffusion,  
 R<sub>4</sub> represents a member selected from the group consisting of a hydrogen atom, an alkyl group, an aryl group, and a group rendering fast to diffusion,  
 further R<sub>3</sub> and R<sub>4</sub> together may also represent the atoms necessary for completing an aromatic ring system.  
 10 7. Photographic multi-layer color material comprising three silver halide emulsion layers which have different optical sensitivities, and containing in non-migratory form in a member selected from the blue-sensitive silver halide emulsion layer and a non-light-sensitive water-permeable colloid layer adjacent thereto a color coupler for yellow having the general formula:



wherein

R<sub>2</sub> represents a member selected from the group consisting of a hydrogen atom, a halogen atom, a methoxy group, a sulfonic acid group, a sulfonic acid salt group, and a group rendering fast to diffusion,  
 R<sub>3</sub> represents a member selected from the group consisting of a hydrogen atom, an alkyl group, an aryl group, and a group rendering fast to diffusion,  
 R<sub>4</sub> represents a member selected from the group consisting of a hydrogen atom, an alkyl group, an aryl group, and a group rendering fast to diffusion,  
 Y represents a bivalent radical, and  
 35 R' represents a sulphonated aromatic radical.

#### References Cited

##### UNITED STATES PATENTS

|    |           |         |                        |           |
|----|-----------|---------|------------------------|-----------|
| 40 | 2,895,825 | 7/1959  | Pelz et al. -----      | 96—56.6   |
|    | 3,008,827 | 11/1961 | Jaeken -----           | 96—100    |
|    | 3,056,674 | 10/1962 | Hoffstadt et al. ----- | 96—100    |
|    | 2,863,874 | 12/1958 | Gregory -----          | 260—306.8 |
|    | 3,124,588 | 3/1964  | Reisner -----          | 260—306.8 |
| 45 | 2,933,391 | 4/1960  | Feniak et al. -----    | 96—100    |
|    | 2,983,608 | 5/1961  | Beavers -----          | 96—100    |

##### OTHER REFERENCES

Glafkides: "Photographic Chemistry," vol. 2, page 606, Fountain Press, London (1960).

J. TRAVIS BROWN, Primary Examiner.

NORMAN G. TORCHIN, Examiner.